

Sept. 9, 1952

H. A. WHEELER

2,610,250

ELECTROMAGNETIC-WAVE ENERGY-ABSORBING MATERIAL

Filed Nov. 5, 1946

FIG. 1



FIG. 2



FIG. 3



FIG. 4



INVENTOR,

HAROLD A. WHEELER,

BY

*Karyl B. Page*

ATTORNEY.

## UNITED STATES PATENT OFFICE

2,610,250

ELECTROMAGNETIC-WAVE ENERGY-  
ABSORBING MATERIALHarold A. Wheeler, Great Neck, N. Y., assignor to  
Hazeltine Research, Inc., Chicago, Ill., a corpora-  
tion of Illinois

Application November 5, 1946, Serial No. 707,787

5 Claims. (Cl. 178—44)

1

The present invention relates to a material adapted to translate an electromagnetic wave and, particularly, to such a material adapted to be interposed in a wave-propagation path and to absorb energy from the wave propagated therethrough. In greater particularity, the invention relates to an electromagnetic-wave energy-absorbing material adapted to absorb substantial amounts of wave energy in small space, yet one having a wave impedance which is substantially purely resistive.

It frequently is desirable to translate an electromagnetic wave along a wave-propagation path which presents to the wave a substantially purely resistive wave impedance yet is capable of dissipating substantial amounts of wave energy. In such cases, it may be desirable to absorb all or part of the wave energy. In the former category may be classified wave-energy "terminating loads" and in the latter wave-energy attenuators.

Dissipation of either the electric-field or magnetic-field energy of a translated wave, however, causes a reactive component to appear in the otherwise purely resistive wave impedances of the wave-propagation path. The amount of the reactive component is proportional to the rate of attenuation per wave length of the translated wave.

In all such wave energy-absorbing arrangements, it has heretofore proven exceedingly difficult to effect the desired wave-energy dissipation without at the same time causing at least some, and frequently a substantial amount, of wave-energy reflection by virtue of the presence of the energy-absorbing material utilized. Such reflection occurs if the wave impedance of the medium is not purely resistive but has a reactive component.

One prior proposed arrangement for dissipating the energy of an electromagnetic wave utilizes the so-called "lossy" coaxial transmission line. This line includes at least a conductor having substantial resistance or a dielectric material having substantial dissipation regarded as shunt conductance. To avoid reflection of wave energy at the input terminals of the line, the line is caused to have a substantially purely resistive input impedance by making its rate of attenuation per wave length so small that the resulting reactive component of its wave impedance is negligible. That is, such lines have heretofore been designed for a small rate of attenuation so as to reduce the reactive component below a permissible tolerance. No attempt has been made to balance the two kinds of reactive components

6 caused by the electric-field and magnetic-field energy dissipations. It is therefore necessary to employ a great length of "lossy" line where it is essential that a substantial part or all of the wave energy applied thereto is to be dissipated in the line. The resulting bulk and expense of such a long line is a serious disadvantage in many applications.

10 When the frequency of a wave signal becomes so high that transmission lines may no longer be conveniently used for wave propagation, a hollow conductor having parameters selected with relation to the wave length of the wave is conveniently used for this purpose. Energy-absorbing arrangements heretofore proposed for wave guides are in the nature of strips of dielectric material or bodies of sand, either of which is coated or impregnated with a resistive material such as colloidal graphite. The material is conveniently molded or otherwise shaped into a configuration so selected as to minimize reflection of wave energy caused by the presence of the material in the wave-propagation path. This result is accomplished by providing a rate of attenuation per wave length which is tapered from a low value to a high value. It is very difficult to avoid such reflection in limited space, however, regardless of the selected shape of the material, and this fact has heretofore necessitated the use of some additional means for compensating or avoiding the effect of the reflected wave energy. Substantial values of energy dissipation in limited space necessitate large values of energy attenuation per wave length of the translated wave, so large in fact that dissipation of either the electric-field energy or the magnetic-field energy by itself would cause a detrimental amount of reactive component in the wave impedance presented to the translated wave. It may be mentioned that reflected wave energy, unless compensated as mentioned, is very undesirable in many applications for the reason that it impairs the operation of wave-signal apparatus located along the wave-propagation path at points preceding the point of wave-energy reflection. Additionally, it is apparent that wave-energy reflection impairs the efficiency of those arrangements which are intended to absorb all of the wave energy supplied thereto.

15 It is an object of the present invention, therefore, to provide a new and improved electromagnetic-wave energy-absorbing material which avoids one or more of the disadvantages and limitations of prior such materials.

20 It is a further object of the invention to provide a new and improved electromagnetic-wave

25 30 35 40 45 50

energy-absorbing material which is capable of absorbing very substantial amounts of wave-signal energy in exceptionally small space yet one which has a wave impedance substantially purely resistive.

It is an additional object of the invention to provide an electromagnetic-wave energy-absorbing material, adapted to be interposed in a non-dissipative wave-propagation path having a predetermined wave impedance, which is capable of absorbing substantial amounts of wave energy yet has a substantially purely resistive wave impedance equal to that of the non-dissipative wave-propagation path.

In accordance with a particular form of the invention, an electromagnetic-wave energy-absorbing material, adapted to be interposed in a wave-propagation path of which at least a portion has a predetermined ratio of dielectric constant to magnetic permeability for a predetermined mode of wave propagation therethrough comprises a quantity of dielectric material and a quantity of high-conductivity material consisting of particles having at least one dimension which is small in relation to the wave length of an electromagnetic wave to be translated thereby. The relative quantities of the aforesaid dielectric and high-conductivity materials are so proportioned with relation to their dielectric constants and magnetic permeabilities as to provide, for the above-mentioned predetermined mode of wave propagation therethrough and along the aforesaid portion of said path, a ratio of effective dielectric constant to effective magnetic permeability for the energy-absorbing material substantially equal to the above-mentioned predetermined ratio. The energy-absorbing material includes a substantial quantity of high-resistance material dispersed in at least a portion of the aforesaid dielectric material consisting of particles having at least one dimension small in relation to the wave length of the translated wave and effective to cause substantial dissipation of the electric energy of the translated wave.

For a better understanding of the present invention, together with other and further objects thereof, reference is had to the following description taken in connection with the accompanying drawing, and its scope will be pointed out in the appended claims.

Referring now to the drawing, Fig. 1 illustrates an electromagnetic-wave energy-absorbing material embodying the present invention and utilized in a particular application; Figs. 2 and 3 illustrate modified forms of the invention; and Fig. 4 illustrates the use of the material embodying the invention in another application.

Referring now more particularly to Fig. 1, there is illustrated a high-frequency electromagnetic-wave energy-absorbing material embodying the present invention in a particular form. Energy-absorbing material 10 embodying the present invention is here shown by way of example as utilized in a coaxial transmission line which includes an outer conductor 11 and an inner conductor 12, the latter being supported by the material 10 in coaxial relation with the conductor 11. The transmission line 11, 12 is essentially a wave-signal propagating device adapted to effect propagation of high-frequency electromagnetic waves along a predetermined propagation path between the conductive surfaces of the conductors 11, 12.

The energy-absorbing material 10 is thus interposed in the wave-propagation path and com-

prises three materials; namely, dielectric material, conductive material and resistive material. The conductive material is dispersed in at least a portion of the dielectric material and is of such configuration and conductivity as to cause dissipation of wave energy in substantial amount in a given manner with reference to the density of the magnetic energy of an electromagnetic wave translated through the energy-absorbing material 10. This conductive material may be in the form of conductive particles, for example combined iron or any comminuted conductive material such as copper, brass, silver, aluminum, etc. Iron, of course, is recognized not only as a conductive material but also as a magnetic material in that it has a coefficient of magnetic permeability greater than that of free space. Copper, silver, or the like are conductors not referred to as magnetic materials, but particles thereof cause dissipation in accordance with the density of magnetic energy in a wave. Usually the given manner of energy dissipation to which reference was last made is a proportional one. That is, the dissipation of the wave energy by the conductive material is usually proportional to the density of the magnetic energy of the translated electromagnetic wave.

The particles of the conductive material of the energy-absorbing material 10 are individually insulated and may be held together in a compact mass by a suitable dielectric binder.

The resistive material of the energy-absorbing material 10 also is dispersed in at least a portion of the dielectric material previously mentioned and is of such configuration and resistivity as to cause dissipation of wave energy in substantial amount and in the aforementioned given manner with reference to the density of the electric field of the wave translated through the energy-absorbing material 10. This resistive material also may be in the form of individually insulated particles, for example powdered carbon or graphite, one preferred form being colloidal graphite. The relative concentrations of the conductive and resistive materials are so proportioned as to cause substantially equal amounts of the magnetic-field-energy dissipation and the electric-field-energy dissipation of the translated electromagnetic wave. This causes the wave impedance of the energy-absorbing material 10 to be substantially purely resistive, because the two kinds of dissipation tend to cause opposite reactive components in the wave impedance.

The dielectric, conductive and resistive materials may be mixed together in the proper quantities into an isotropic mixture and are then molded, cast or compressed into a rigid mass of configuration suitable for the use intended. Thus in a coaxial transmission line of the type shown in Fig. 1, the energy-absorbing material 10 may, after proper mixing of its ingredient materials, be molded or compressed into apertured cylindrical blocks or discs suitable for insertion between the line conductors 11, 12. Alternatively, the material 10 may be extruded upon the line conductor 12 after which the line conductor 11 may be applied over the material 10 as a woven braid or tube. When the energy-absorbing material 10 is formed as described, the particles of conductive and resistive materials are held in solid suspension in, and dispersed throughout, the dielectric material so that the latter provides individual insulation for the particles.

The particle size and particle spacing for an isotropic medium must be much less than a radian

length of the translated wave and, of course, the density must be substantially uniform throughout the medium. Particles having a radius of the order of one radian length in the material of the particle are perhaps somewhere near the optimum. In the case of metals and graphite, one radian length is equal to the depth of penetration in the material. Where the material 10 is not isotropic, as a laminated form of the material presently to be described, the particles of conductive and resistive materials should nevertheless have some dimension much less than a wave length of the translated wave signal. For magnetic material, the dimension along the vector of the electrical field of the wave should be small; for resistive material, the dimension along the vector of the magnetic field should be small. The term "particle" as used in the present specification and claims is thus intended to mean pieces of material having sizes small in relation to the wave length of the translated wave signal. For very long wave lengths, the magnetic material might thus be scrap iron, sheets of conductive material, and the like.

In the operation of a transmission line of the type illustrated, electromagnetic wave energy when applied to one end of the line is propagated between the line conductors and travels along the line. The magnetic field of the electromagnetic wave sets up eddy currents in the conductive particles of the material 10 and these currents dissipate some of the magnetic-field energy of the translated wave. The wave thus experiences what may be considered equivalent to a series resistance to its propagation through the material 10. The particles of resistive material included in the energy-absorbing material 10 cause, on the other hand, dissipation of some of the electric-field energy of the translated wave so that the resistive material may be considered equivalent to a shunt conductance between the line conductors 11, 12.

In this type of transmission line, it may be desirable to use such quantities of the dielectric, conductive and resistive materials as to provide a desired ratio of effective inductance to effective capacitance for the line, in which case the invention contemplates a relative concentration of conductive and resistive particles to provide a substantially equal ratio of equivalent series resistance to equivalent shunt conductance. When this is done, the transmission line has a wave impedance which is substantially purely resistive. This result is obtained over a wide range of electromagnetic-wave frequencies if the particles are sufficiently small and closely packed. Thus if the particles are so small that the radius of each particle is less than one radian length in the material of the particle, the resulting attenuation caused by the particle is proportional to the square of the frequency. If both kinds of attenuation are obtained by particles small enough to meet this requirement, it follows that both kinds of attenuation are proportional to the square of the frequency and, therefore, the equality of the electric field and magnetic field dissipations is maintained over a large frequency range. It fails only to the extent that other causes of attenuation become more important at lower frequencies, such as the resistance of the conductor in a transmission line, the power factor of the dielectric binder, etc. When the material 10 has a purely resistive wave impedance, it is capable of dissipating a large part of the electro-

magnetic-wave energy in a small distance without causing reflection.

It frequently is desirable that the energy-absorbing material of the present invention be interposed in a wave propagation path of which at least a portion has a predetermined ratio of dielectric constant to magnetic permeability which determines its wave impedance. Such a path may be non-dissipative and so have a purely resistive wave impedance. This need may occur, for example, when a transmission line of the type shown in Fig. 1 is coupled to a transmission line which utilizes an air dielectric between its conductors. An air-dielectric line has a unity ratio of its dielectric constant to magnetic permeability, if both are expressed relative to free space. If this ratio of dielectric constant to magnetic permeability is not maintained along the entire length of the wave-propagation path, reflections of wave energy occur at those points where there is experienced a change of the ratio mentioned. This is undesirable in many applications for well-known reasons.

Fig. 2 illustrates a form of transmission line of the balanced type having spaced conductors 11, 12. The energy-absorption material 10' used between the line conductors has such composition that most desired ratios of dielectric constant to magnetic permeability may be readily obtained. The method here shown of forming the material 10' for use in a balanced line may also be utilized for a coaxial line of the Fig. 1 type. The material 10' here includes a layer of dielectric material 13 having a lamination thickness  $a_1$ , a dielectric constant  $k_1$ , and a coefficient of magnetic permeability  $\mu_1$ . It also includes a contiguous layer of conductive material 14 in the form of individually insulated conductive particles held together by a suitable dielectric binder. This layer of conductive material 14 has a lamination thickness  $a_2$ , a constant  $k_2$ , and a magnetic permeability  $\mu_2$ . An electromagnetic wave has its electric and magnetic fields normal to each other. A wave of this type is propagated through the material 10' with such polarization that the magnetic field  $H$  is parallel to the layers of the materials 13, 14 and the electric field  $E$  is normal to the layers, as indicated by the arrows  $H$  and  $E$  in Fig. 2.

The laminated construction here utilized is disclosed and claimed in applicant's copending applications Serial No. 563,716, filed November 16, 1944, now Patent No. 2,508,479, issued May 23, 1950, entitled "High-Frequency Electromagnetic-Wave Translating Arrangement," and Serial No. 563,715, filed November 16, 1944, now Patent 2,511,610, issued June 13, 1950, entitled "High-Frequency Electromagnetic-Wave Translating Element," both assigned to the same assignee as the present application. As there explained, the thickness  $a_1$  of the layer of dielectric material 13 and the thickness  $a_2$  of the layer of conductive material 14 are selected in relation to the dielectric constants  $k_1$  and  $k_2$  and magnetic permeabilities  $\mu_1$  and  $\mu_2$  as to provide for the material 10' a ratio of effective dielectric constant to effective magnetic permeability of the desired value. For reasons explained in applicant's aforementioned copending applications, the maximum lamination thickness of the dielectric material 13 and of the conductive material 14 should be much less than one radian length of the translated electromagnetic wave. As in the arrangement of Fig. 1, resistive material in the form of particles 75 is dispersed in either or both of the dielectric ma-

terial 13 and conductive material 14. Also as in Fig. 1, the quantity of the resistive material is such as to cause an amount of electric-field-energy dissipation equal to the amount of magnetic-field-energy dissipation caused by the magnetic conductive material during the propagation of the electromagnetic wave through the material 10'.

Fig. 3 illustrates an energy-absorbing material 10'' which is essentially similar to that of Fig. 2, similar elements and materials being designated by similar reference numerals, except that the material 10'' is formed of alternating laminations of dielectric material 13 and conductive material 14 having quantities relatively proportioned as in Fig. 2 to attain a desired ratio of effective dielectric constant to effective magnetic permeability. As in Fig. 2, the maximum lamination thickness of the dielectric and conductive materials should be much less than one radian length of the translated wave signal.

When the energy-absorbing material of the present invention is interposed in a wave-propagation path and provides unity ratio of the effective dielectric constant to effective magnetic permeability as is characteristic of free space, the wave-propagation velocity through the material is less than that of free space. Fig. 4 represents an application of the present invention in which it is desired that the wave-propagation path through the portion thereof occupied by the energy-absorbing material have an effective electrical length greater than its physical length by virtue of the reduced propagation velocity mentioned. In this arrangement, the energy-absorbing material 10''' is of cylindrical cross section and is positioned on the inner conductor 12 of the transmission line 11, 12. Assuming the line to be air filled, uniformity of impedance along the transmission line is maintained when the radial thickness  $x$  of the material 10''' has a value given by the relation:

$$x = \frac{\mu + \frac{1}{k} - 2}{(\mu - 1) \left( 1 - \frac{1}{k} \right)} \quad (1)$$

where:

$\mu$ =the effective magnetic permeability of the material of element 10'''

$k$ =the effective dielectric constant of the material of element 10'''.

The length of the material 10''' is selected, of course, to provide the desired increase of electrical length of the transmission line. As before, the relative concentrations of the conductive and resistive materials provided in the energy-absorbing material 10''' are such as to cause substantially equal amounts of the magnetic-field-energy dissipation and electro-field-energy dissipation so that the wave impedance of the transmission line is substantially purely resistive.

From the above description of the invention, it will be apparent that an electromagnetic-wave energy-absorbing material embodying the present invention is adapted to provide, in a limited space, substantial absorption of electromagnetic-wave energy yet is one which has a substantially purely resistive wave impedance and thus does not cause reflection of wave-signal energy. The magnitude of attenuation of which the material of the present invention is capable may be as high as 100 decibels or higher per wave length, while yet maintaining the wave impedance of the ma-

terial substantially purely resistive. For example, it is easily possible to attain with the material of the present invention an attenuation of about one napier per radian length or 55 decibels per wave length while maintaining the net reactive component of wave impedance of the material to within a few per cent. of the resistive component; with only one kind of dissipation, that is dissipation of only the electric-field energy or the magnetic-field energy of the translated wave signal, this would yield in the absence of the present invention a reactive component of the same order of magnitude as the resistive component of wave impedance. The advantages of attaining such large attenuation in so limited a space and while maintaining a substantially purely resistive wave impedance are at once apparent. There is the further advantage with the energy-absorbing material of the present invention that its wave impedance may be easily made substantially equal to that of a non-dissipative wave-propagation path in which the material may be inserted or of which it may be a component part.

While there have been described what are at present considered to be the preferred embodiments of this invention, it will be obvious to those skilled in the art that various changes and modifications may be made therein without departing from the invention, and it is, therefore, aimed in the appended claims to cover all such changes and modifications as fall within the true spirit and scope of the invention.

What is claimed is:

1. An electromagnetic-wave energy-absorbing material, adapted to be interposed in a wave-propagation path of which at least a portion has a predetermined ratio of dielectric constant to magnetic permeability for a predetermined mode of wave propagation therethrough comprising: a quantity of dielectrical material; a quantity of high-conductivity material consisting of particles having at least one dimension which is small in relation to the wave length of an electromagnetic wave to be translated thereby; the relative quantities of said materials being so proportioned with relation to their dielectric constants and magnetic permeabilities as to provide, for said predetermined mode of wave propagation therethrough and along said portion of said path, a ratio of effective dielectric constant to effective magnetic permeability for said energy-absorbing material substantially equal to said predetermined ratio; and a substantial quality of high-resistance material dispersed in at least a portion of said dielectric material consisting of particles having at least one dimension small in relation to the wave length of said translated wave and effective to cause substantial dissipation of the electric energy of said translated wave.

2. An electromagnetic-wave energy-absorbing material adapted to be interposed in a wave-propagation path of which at least a portion has a predetermined ratio of dielectric constant to magnetic permeability and a substantially purely resistive wave impedance for a predetermined mode of wave propagation therethrough comprising: a quantity of dielectric material; a substantial quantity of high-conductivity material consisting of individually insulated particles having maximum dimensions which are small in relation to the wave length of an electromagnetic wave to be translated thereby and effective to cause substantial dissipation of the magnetic energy of said translated wave; the relative quantities of said materials being so proportioned with

relation to their dielectric constants and magnetic permeabilities as to provide, for said predetermined mode of wave propagation therethrough and along said portion of said path, a ratio of effective dielectric constant to effective magnetic permeability for said energy-absorbing material substantially equal to said predetermined ratio; and a substantial quantity of high-resistance material dispersed in at least a portion of said dielectric material consisting of individually insulated particles having maximum dimensions small in relation to the wave length of said translated wave and effective to cause substantial dissipation of the electric energy of said translated wave.

3. An electromagnetic-wave energy-absorbing material, adapted to be interposed in a wave-propagation path of which at least a portion has a predetermined ratio of dielectric constant to magnetic permeability and a substantially purely resistive wave impedance for a predetermined mode of wave propagation therethrough comprising: a quantity of dielectric material; a quantity of high-conductivity material consisting of individually insulated particles having maximum dimensions of the order of one radian length of an electromagnetic wave to be translated thereby; the relative quantities of said materials being so proportioned with relation to their dielectric constants and magnetic permeabilities as to provide, for said predetermined mode of wave propagation therethrough and along said portion of said path, a ratio of effective dielectric constant to effective magnetic permeability for said energy-absorbing material substantially equal to said predetermined ratio; and a substantial quantity of high-resistance material dispersed in at least a portion of said dielectric material consisting of individually insulated particles having maximum dimensions of the order of one radian length of said translated wave and effective to cause substantial dissipation of the electric energy of said translated wave.

4. An electromagnetic-wave energy-absorbing material adapted to be interposed in a wave-propagation path of which at least a portion has a predetermined ratio of dielectric constant to magnetic permeability for a predetermined mode of wave propagation therethrough comprising: at least one layer of a quantity of dielectric material; at least one layer of a quantity of high-conductivity material contiguous to said first-mentioned layer and comprising individually insulated particles having maximum dimensions which are small in relation to the wave length of an electromagnetic wave to be translated thereby; the relative quantities of said materials being so proportioned with relation to their dielectric constants and magnetic permeabilities as to provide, for said predetermined mode of wave propagation

therethrough and along said portion of said path, a ratio of effective dielectric constant to effective magnetic permeability for said energy-absorbing material substantially equal to said predetermined ratio; and a substantial quantity of high-resistance material dispersed in at least a portion of said dielectric material consisting of individually insulated particles having maximum dimensions small in relation to the wave length of said translated wave and effective to cause substantial dissipation of the electric energy of said translated wave.

5. An electromagnetic-wave energy-absorbing material, adapted to be interposed in a wave-propagation path of which at least a portion has a predetermined ratio of dielectric constant to magnetic permeability for a predetermined mode of wave propagation therethrough comprising: at least one layer of a quantity of dielectric material having a maximum thickness much less than one radian length of an electromagnetic wave to be translated thereby; at least one layer of a quantity of high-conductivity material, contiguous to said first-mentioned layer, comprising individually insulated particles having maximum dimensions which are small in relation to the wave length of said translated wave and having a maximum thickness much less than one radian length of said translated wave; the relative quantities of said materials being so proportioned with relation to their dielectric constants and magnetic permeabilities as to provide, for said predetermined mode of wave propagation therethrough and along said portion of said path, a ratio of effective dielectric constant to effective magnetic permeability for said energy-absorbing material substantially equal to said predetermined ratio; and a substantial quantity of high-resistance material dispersed in at least a portion of said dielectric material consisting of individually insulated particles having maximum dimensions small in relation to the wave length of said translated wave and effective to cause substantial dissipation of the electric energy of said translated wave.

HAROLD A. WHEELER.

#### REFERENCES CITED

The following references are of record in the file of this patent:

#### UNITED STATES PATENTS

| Number    | Name   | Date          |
|-----------|--------|---------------|
| 1,741,582 | Power  | Dec. 31, 1929 |
| 2,343,040 | Allen  | Feb. 29, 1944 |
| 2,393,541 | Kohler | Jan. 22, 1946 |
| 2,412,805 | Ford   | Dec. 17, 1946 |
| 2,423,396 | Linder | July 1, 1947  |
| 2,464,006 | Tiley  | Mar. 8, 1949  |